

# UNITED STATES PATENT OFFICE.

ADOLPHE SEGAY, OF WARE, ENGLAND.

## EXPLOSIVE.

1,280,563.

Specification of Letters Patent. Patented Oct. 1, 1918.

No Drawing.

Application filed August 7, 1917. Serial No. 184,870.

To all whom it may concern:

Be it known that I, ADOLPHE SEGAY, a citizen of the French Republic, residing in Ware, Hertfordshire, England, have invented certain new and useful Improvements in Explosives, of which the following is a specification.

This invention is for improvements in explosives and it relates more particularly to explosives which contain a silicid of an alkaline earth metal and has an ammonium nitrate base.

It has been found that such explosives cannot be usefully compressed to any great degree. As is well-known the action of an explosive usually is improved by compression, but it is found that explosives of the class mentioned do not explode satisfactorily if compressed; for example, a known explosive of this class composed as follows:—

|                  |       |
|------------------|-------|
| Ammonium nitrate | 78.20 |
| Trinitrotoluene  | 8.00  |
| Calcium silicid  | 13.80 |

has a specific gravity when loose of .8. When compressed in the ordinary manner into a cartridge case, it has a specific gravity of 1.0 and it can be advantageously compressed so that its specific gravity reaches 1.25 but when compressed beyond this, it does not explode satisfactorily. The fact that an explosive of the kind under consideration cannot be compressed to raise its specific gravity above 1.25 has two disadvantages, (1) that the usual means of increasing the efficiency of the explosive by compression is not available for this explosive, and (2) that when compressed to a specific gravity of 1.25 the blocks or sticks thus produced are not sufficiently hard to enable them to be readily handled for wrapping; they are also more hygroscopic than would be the case if they were subjected to greater pressure. Moreover, the specific gravity 1.25 is the maximum at which this explosive is able to detonate, and in ordinary practice a specific gravity of 1.15 is the maximum employed for the ammonium nitrate explosives.

It has been found, however, that if the proportion of the alkaline earth silicid is increased relatively to the oxygen carrier, such as the ammonium nitrate, a more powerful explosive is obtained and the explosive can be advantageously compressed so that it becomes hard enough to handle easily

and is less hygroscopic than that heretofore manufactured.

This invention therefore consists in the provision of an explosive of the kind described, characterized by the proportion of the alkaline earth silicid (for example calcium silicid) being in excess of what would ordinarily be calculated as necessary to obtain what heretofore has been known as the best proportions corresponding to a complete combustion, i. e., an explosive containing such a proportion of combustible material that the oxygen coming from an oxygen carrier such as the ammonium nitrate is in a sufficient quantity to oxidize the silicid and burn all the carbon existing in the explosive to carbon dioxid and all the hydrogen to water.

It is also necessary to introduce into the composition of the explosive a small quantity of a substance which may be detonated by itself, to start combustion of the silicid and to enable it to be compressed. As examples of substances which may be employed for this purpose may be mentioned trinitrotoluene, tetranitro-methylanilin, hexanitrodiphenylamin, nitroglycerin, and tetranitranilin, and the quantity may vary from 6 to 10% according to the nature of the material employed and its detonating power.

An explosive according to the present invention has the following composition:—

|                                                                            |      |    |
|----------------------------------------------------------------------------|------|----|
| Ammonium nitrate                                                           | 66.0 | 90 |
| Tetranitro-methylanilin, or any explosive which may be detonated by itself | 7.0  |    |
| Calcium silicid                                                            | 27.0 |    |

It will be seen that in this formula, the silicid is in considerable excess of what would be ordinarily calculated as necessary for the proper utilization of the oxygen carrier, i. e. the nitrate, and such a mixture is found to give a 10% increase of explosive force, when loose, as compared with explosives of the same class as heretofore manufactured, and moreover it can be compressed to a specific gravity of 1.45 or above this if desired. At 1.45 the material is sufficiently solid to permit of its being easily handled for wrapping. The higher compression of course also renders the explosive less hygroscopic and as it can be easily handled it can be rendered still less liable to absorb moisture by known methods such as dipping it in paraffin-wax or otherwise

treating it externally. The proportion of calcium silicid can advantageously be carried as high as 27.0% when the tetranitromethylanilin or other explosive which will detonate by itself can be reduced as low as 6.0%.

It will be seen that through being able to compress the explosive, say to 1.45 specific gravity instead of 1.15, a given quantity of explosive is made to occupy a less space than it would when less compressed and therefore it does not require so much paper and paraffin wrapping. This means that some of the nitrate which before was absorbed in consuming the paper and paraffin wrapping is now free and therefore more silicid can be added to usefully cooperate with this freed amount of nitrate, but apart from this it is found that if the quantity of silicid is increased beyond what is theoretically expected to be the right amount an explosive of higher power is obtained, as already stated.

The most powerful form of the explosive appears to be that in which the proportion of combustible material is such that, once the metal is oxidized, the whole of the carbon is burned to carbon monoxide and half of the hydrogen to water. If this proportion is exceeded, a deposit of carbon is found in the products of combustion, and the power of the explosive is decreased.

In an explosive of the kind described in the specification there is present a much larger quantity of combustible substance than in previously known explosives of this class. So large a quantity of combustible substance in these previously known explosives would bring about the production of too large a quantity of carbon monoxide, but in an explosive according to the present invention the amount of this gas produced is not more than is usual with ordinary ex-

plosives. That the quantity is small is due to two reasons:—

(1) Because as explained above the explosive according to the present invention can be compressed whereby the quantity of paper and paraffin wrapping is reduced; and

(2) The total quantity of carbon present in the composition of the explosive is small.

What I claim as my invention and desire to secure by Letters Patent is:—

1. An alkaline-earth silicid explosive wherein the proportion of the alkaline-earth silicid is in excess of what would ordinarily be calculated as necessary to provide an explosive containing what heretofore has been known as the best proportions for producing complete combustion, that is, an explosive which contained such a proportion of combustible material that the oxygen coming from the oxygen-carrier was in sufficient quantity to oxidize completely the silicid and burn all the carbon existing in the explosive to carbon dioxide and all the hydrogen to water.

2. An explosive containing approximately 66.0 parts of an oxygen-carrier, 7.0 parts of an explosive which may be detonated, and 27.0 parts of an alkaline-earth silicid.

3. An explosive of the kind described characterized by the proportion of the alkaline earth silicid being so much in excess of what would ordinarily be calculated as necessary for the proper utilization of the oxygen carrier of the explosive that as soon as the metal is oxidized approximately the whole of the carbon is converted to carbon monoxide and approximately half of the hydrogen to water.

In testimony whereof I have signed my name to this specification.

ADOLPHE SEGAY.